

1

3,070,576

## COMPLEX METAL SALTS OF ALKYLPHENOL-ALDEHYDE CONDENSATION PRODUCTS AND METHOD FOR PREPARING SAME

George W. Munns, Jr., West Deptford Township, Gloucester County, Ferdinand P. Otto, Woodbury, and Francis M. Seger, Mount Ephraim, N.J., assignors to Socony Mobil Oil Company, Inc., a corporation of New York

No Drawing. Original application Apr. 24, 1958, Ser. No. 730,528, now Patent No. 3,014,868, dated Dec. 26, 1961. Divided and this application Apr. 26, 1960, Ser. No. 24,666

14 Claims. (Cl. 260—53)

This invention relates to a new class of additives useful as motor oil detergents and to a method for preparing these additives.

It is well known that lubricating oils tend to deteriorate under the conditions of use in present day diesel and automotive engines with attendant formation of sludge, lacquer and resinous materials which adhere to the engine parts, particularly the piston ring grooves and skirts, thereby lowering the operating efficiency of the engine. To counteract the formation of these deposits, certain chemical additives have been found which when added to lubricating oils have the ability to keep the deposit-forming materials suspended in the oil so that the engine is kept clean and in efficient operating condition for extended periods of time. These addition agents are known in the art as detergents of dispersants. Metal organic compounds, particularly metal salts of organic acids, are useful in this respect. It has been shown furthermore that such salts prepared by processes which enable the incorporation of "excess" amounts of metal therein, i.e., amounts over and above that required to form normal salts, exhibit markedly improved ability as detergents for lubricating oils, particularly oils employed in the lubrication of engines using high sulfur-content fuels. Methods whereby the advantageous excess amounts of metal are incorporated into the detergent salts are, therefore, of great value to the art. These high metal-content salts are generally termed "complex" salts for the reason that the excess metal is believed to be incorporated therein through some type of complexing mechanism, such as occurs in the formation of Werner Coordination Compounds. The present invention is concerned with the provision of such a process. Thus, by the process of this invention, it is possible to prepare complex metal salts of alkylphenol-formaldehyde condensation products having incorporated therein from about 50 to about 100% excess metal and which are highly effective motor oil detergents. These salts have also been found to be effective antioxidants for such oils.

As far as is known the high metal-content "complex" salts of this invention have not been produced heretofore and they are therefore, believed to be new compositions of matter. Accordingly, it is the primary object of this invention to provide a new process for the preparation of high metal-content salts of alkylphenol-formaldehyde products.

It is a further object of the invention to provide a new class of high metal-content salts. It is a still further object to provide mineral lubricating oil compositions of improved detergent and antioxidant character said compositions containing the new high metal-content "complex" salts herein disclosed. Other and further objects of the invention will be apparent from the following description thereof.

As has been indicated, various processes for preparing high metal-content salts have recently been developed in the art. It has been shown, however, that the success of

2

such methods depends not only upon the conditions and techniques employed but is apt to vary with the particular metal sought to be incorporated into the complex salt product. Thus, it has been found that a method whereby the complex salt of one metal can be successfully prepared is oftentimes unsuccessful when applied to the preparation of a salt of a different metal. It is seen then that the metals, even metals of the same group in the periodic table, are not equivalent in their ability to form high metal-content complex salts.

It has been found that the method of the present invention can be successfully employed to prepare high metal-content salts of the metals barium, strontium, sodium, and potassium, but is not capable of producing complex salts having any substantial excess of other metals such as calcium, magnesium and zinc. This invention, therefore, is directed specifically to the preparation of complex salts of barium, strontium, sodium and potassium, the only metals which have been found to provide such salts by the application of the method.

Broadly stated, the method of the invention involves the interaction of (a) an alkylphenol of a defined type, as set forth hereinafter, (b) formaldehyde, (c) a carboxylic acid selected from formic acid and hydroxyacetic (glycolic) acid and (d) a metal hydroxide of barium, strontium, sodium or potassium, in a suitable solvent medium, such as a mineral oil, at a temperature of from about 40 to about 85° C. followed by dehydration to remove water of reaction and final filtration to remove insolubles, such as excess salt reagent and the like. It has been found that other carboxylic acids, such as acetic acid, and dicarboxylic acids, such as oxalic acid, do not provide the desired complex salts when used in the process of the invention as do formic and glycolic acids.

35 A modification of the process involves subjecting the reaction mixture, prior to final filtration, to treatment with carbon dioxide. This treatment, however benefits the process only with respect to the preparation of the barium and strontium salts of the invention and is not of advantage when applied to the preparation of the sodium and potassium salts, as will be explained hereinafter.

40 A preferred procedure for carrying out the process of the invention is as follows. The alkylphenol, formaldehyde, formic acid or hydroxyacetic acid and metal hydroxide reagents are brought together in a suitable solvent, such as mineral oil. The solvent mixture is then heated with stirring to a moderately elevated temperature, say, about 40 to about 85° C. and maintained at this temperature for about one hour. Thereafter, the temperature of the reaction mixture is raised to at least about 150° C., preferably about 200° C., and maintained at this temperature until all of the water of reaction has been driven off. The hot reaction mixture is then filtered to remove insoluble material, such as excess salt reagent. As indicated previously, in the preparation of the barium and strontium complex salts the reaction mixture, prior to filtration, may be treated with carbon dioxide. In the case of the barium and strontium salts, it has been found that the carbonation effects a substantial increase in the metal contents of the product salts and at the same time increases the fluidity of the product mixture so that filtration and handling of the product is greatly facilitated. Furthermore, it has been found that the carbonation treatment neutralizes the strong base constituents present in the barium and strontium complex salts without, however, reducing their high reserve alkalinity, which is particularly desirable if the salts are to be added to lubricating oils for use in engines burning high sulfur-content fuels. With respect to the preparation of the sodium and potassium complex salts, however, it has been found that the carbonation treatment tends to reduce rather than increase the metal contents of the product salts. For this

reason, and because these salts are not highly viscous, the use of the carbonation step is not prescribed for the preparation of these salts.

Although it is generally preferred to use a mineral lubricating oil as the solvent, it will be appreciated that other solvents may be used in the process of the invention. Thus, any inert hydrocarbon solvent having a sufficiently high boiling point (above about 150° C.), such as a naphtha fraction or the like may be used. In such case, the solvent may be removed from the product salt by distillation or the product salt may be retained therein for convenience in handling, shipping, etc. However, the use of a mineral lubricating oil as solvent is preferred as it need not be removed from the product prior to use, the concentrated oil solution being directly blendable with the lubricating oil stock desired to be fortified by addition of the complex salt product thereto.

Although the above-described procedure for carrying out the process of the invention is preferred, other modes of operation are entirely satisfactory and may be employed. Thus, the order in which the reactants are brought together may be varied as follows: (1) The alkylphenol, formaldehyde and barium hydroxide reagents may be added to the mineral oil solvent and the mixture heated after which the formic or hydroxyacetic acid is added; (2) The alkylphenol, formaldehyde and formic or hydroxyacetic acid may be added to the mineral oil and the mixture heated after which the barium hydroxide is added; (3) The alkylphenol-formaldehyde condensation product can be formed separately after which the barium hydroxide and the acid reagents are added; and (4) The alkylphenol, formaldehyde and barium hydroxide can be added to the oil and the mixture reacted, dehydrated and filtered, after which the acid reagent is added.

Broadly, the ratios of reagents employed in the process of the invention are as follows. For each mole of alkylphenol (a) about 1.3 moles of formaldehyde, (b) from about 0.85 to about 2.0 moles of metal hydroxide when the metal is barium or strontium and from about 1.70 to about 4.0 moles of metal hydroxide when the metal is either sodium or potassium and (c) from about 0.5 to about 1.0 mole of formic or hydroxyacetic acid; the preferred ratios being (a) about 1.0 mole of formaldehyde, (b) about 1.1 moles of either barium or strontium hydroxide and about 2.2 moles of either sodium or potassium hydroxide and (c) about 0.5 mole of formic acid or glycolic acid per mole of alkylphenol.

When the carbonation treatment is employed, the amount of carbonation required is small. Thus, it has been found that the first introduction of carbon dioxide effects a marked improvement in the fluidity of the reaction mass. Generally, however, in order to provide products of reduced strong alkalinity, the carbon dioxide is used in amounts sufficient to incorporate from about 0.1 to about 0.7 mole of carbon dioxide per mol of alkylphenol in the complex salt product.

With respect to the amount of metal hydroxide reagent used in the process, it has been found that the use of amounts higher than those mentioned hereinabove usually results in filtration difficulties.

As already stated, the initial reaction temperature (i.e., prior to the dehydration step) is from about 40 to about 85° C. A reaction time of about one hour at this temperature is generally allowed in order to insure completion of the reaction. For the dehydration step, the temperature of the reaction mixture is increased to above 100° C., and preferably to 150-200° C., due to the fact that at lower temperatures than 150° C. the reaction mixture is apt to be quite viscous. Also the higher dehydration temperatures insure relatively rapid and thorough removal of the water. Also, it is preferred to conduct the carbonation treatment at the 200° C. level as it has been found in the case of the barium and strontium salts that carbonation at this temperature effects about

a 12% increase in the metal content of the complex salt products over that provided by carbonation at 150° C. The time of carbonation will, of course, vary depending upon the size of the reaction mass, the rate of introduction of the carbon dioxide, the efficiency of contacting, etc. Accordingly, although the examples presented hereinafter show carbonation times varying between about 2 and about 8 hours, it should be appreciated that the required carbonation time could be longer or shorter depending upon the type of reactor used, etc.

The alkylphenols suitable for use in the invention comprise the mono-alkyl-substituted phenols in which the alkyl substituent group contains from about 8 to about 18 carbon atoms. Alkylphenols having alkyl substituents of less than 8 carbon atoms generally do not provide complex salts which are oil-soluble. Specific examples of suitable alkylphenols are the following: mono-octyl phenol, mono-nonyl phenol, mono-decyl phenol, mono-dodecyl phenol, mono-tetradecyl phenol, mono-hexadecyl phenol and mono-octadecyl phenol.

It has been found that when dialkyl-substituted phenols are employed in the process of the invention, the metal contents of the salt products are not significantly greater than those of the normal salts. The method of the invention, therefore, is specific to the mono-alkylphenols, although a crude grade of alkylphenols consisting of a mixture of mono- and di-alkylphenols, and containing predominantly mono-alkylphenols, has been found to give complex salt products. The metal contents of these salts, however, are not as high as those obtained using a "commercial" grade of mono-nonyl phenol.

The exact nature of the complex barium salts of the invention is not presently known. Without intending to limit the invention by theoretical considerations, however, it is believed that the salt product is a complex of metal formate, hydroxide, carbonate or bicarbonate bonded to the phenate salt by coordinate bonds of the type found in Werner Coordination Compounds.

The following examples will serve to fully illustrate the invention. In these examples both the percentage metal content (found by actual analysis) and the percentage of "excess" metal (calculated on the basis of the theoretical content of the corresponding normal salt) in each instance are shown for each of the complex salt products. Thus, for example, 100% "excess" means that the metal content of the complex salt product is twice as great as that of the corresponding normal metal salt. In certain of the examples, however, in which the metal content of the product salt was less than the theoretical metal content of the normal salt, the percentage of theoretical metal content ("percent of theory") is shown along with the actual percentage metal content. These latter examples illustrate preparations outside the scope of this invention.

#### EXAMPLE 1

##### Reagents Charged

110 grams (0.5 mole) of nonylphenol  
42 grams (0.5 mole) of formaldehyde (36% solution)  
185 grams (0.58 mole) of barium hydroxide octahydrate  
23 grams (0.5 mole) of formic acid (98%)  
330 grams of conventional paraffin oil (100 sec. at 100° F.)

##### Procedure

All of the materials were mixed in a three-liter, four-neck flask equipped with a mechanical stirrer, thermometer, nitrogen inlet tube, Dean-Stark water take-off and reflux condenser. The reagents were mixed and heated to 50-55° C. for one hour. Nitrogen was then applied, the heat increased and water distilled from the reaction mixture until a temperature of 200° C. was reached. This temperature was maintained for one hour to insure complete dehydration. About 150 grams of this material was removed and filtered through a "Hyflo" (a di-

atomaceous earth filter aid) precoated, electrically heated Buchner funnel to yield a viscous product.

*Product Analysis*

Barium, percent..... 11.69 (86% excess).  
Potentiometric base number..... 87 (total), 53 (strong).

**EXAMPLE 2**

*Procedure*

The remainder of the reaction product prepared in Example 1 was treated prior to filtration for eight hours at 200° C. with a stream of carbon dioxide gas. The resulting material was cooled and filtered in the usual manner yielding a greenish oil of low viscosity.

*Product Analysis*

Barium, percent..... 12.17 (94% excess).  
Potentiometric base number..... 84 (total), 39 (strong).  
Formic acid, percent..... 2.73.  
Carbon dioxide, percent..... 1.40.  
Specific gravity at 26° C..... 1.050.

**EXAMPLE 3**

*Reagents Charged*

- (A) 110 grams (0.5 mole) of nonylphenol  
330 grams of conventional paraffin oil (100 sec. at 100° F.)  
174 grams (0.55 mole) of barium hydroxide octahydrate  
54 grams (0.65 mole) of formaldehyde (36% solution)  
(B) 14.1 grams (0.25 mole) of formic acid (88-90%)  
(C) Carbon dioxide

*Procedure*

All of the materials of group (A) were mixed and heated at 40-60° C. for one hour in a one-liter, four-neck, round-bottom flask equipped with a mechanical stirrer, thermometer, nitrogen inlet tube and Dean-Stark water take-off with reflux condenser. The formic acid (B) was added to this mixture over a twenty minute period at 60-70° C. Water was then removed by distillation until a maximum temperature of 150° C. was reached. This temperature was held for one hour, after which a 100 gram sample was removed and filtered in the normal manner. The remainder of the material was carbonated for 2.5 hours at 200° C. and filtered by the conventional method.

*Product Analysis*

Barium, percent..... 12.30 (96% excess).  
Potentiometric base No..... 83 (total), 19 (strong).  
Kinematic viscosity at 210° F., cs..... 13.34.  
Formic acid, percent..... 1.83.  
Carbon dioxide, percent..... 2.54.  
Specific gravity at 24° C..... 1.053.

**EXAMPLE 4**

*Reagents Charged*

- 550 grams (2.5 moles) of nonylphenol  
1650 grams of conventional paraffin oil (100 sec. at 100° F.)  
870 grams (2.75 moles) of barium hydroxide octahydrate  
208 grams (2.5 moles) of formaldehyde (36% solution)  
70.5 grams (1.25 moles) of formic acid (88-90%)

*Procedure*

The procedure was the same as that described in Example 1 except that a maximum dehydration temperature of 150° C. was used. A sample of the product mixture was withdrawn for use in Example 5. The carbonation was then carried out for 3 hours at 200° C.

*Product Analysis*

Barium, percent..... 12.27 (95% excess).  
Potentiometric base number..... 85 (total), 25 (strong).  
K.V. at 210° F., cs..... 12.00.  
Formic acid, percent..... 1.68.  
Carbon dioxide, percent..... 2.21.  
Specific gravity at 26° C..... 1.051.

**EXAMPLE 5**

*Procedure*

The portion of uncarbonated product retained in Example 4 was carbonated at 150° C. for 2 hours by the conventional procedure.

*Product Analysis*

Barium, percent..... 10.86 (72% excess).  
20 It is seen that the longer carbonation (3 hours) at the higher temperature (200° C.) employed in Example 4 produced a complex salt of higher barium content than obtained in this example.

**EXAMPLE 6**

In this example, a mixture of 20 mole percent of di-nonylphenol and 80 mole percent of nonylphenol was used and gave a satisfactory metal retention.

*Reagents Charged*

- 30 88 grams (0.4 mole) of nonylphenol  
34 grams (0.1 mole) of dinonylphenol  
174 grams (0.55 mole) of barium hydroxide octahydrate  
45 grams (0.55 mole) of formaldehyde (36% solution)  
35 12.6 grams (0.25 mole) of formic acid (88-90%)  
330 grams of conventional paraffin oil (100 sec. at 100° F.)

*Procedure*

40 The same preparative methods were used as noted under Example 1, except that a maximum dehydration temperature of 150° C. was used. The product was treated with CO<sub>2</sub> for two hours at 200° C. by the conventional procedure.

*Product Analysis*

Barium, percent..... 12.94 (109% excess).  
45 Potentiometric base number..... 96 (total), 28 (strong).  
Kinematic viscosity at 210° F., cs..... 16.27.  
Formic acid, percent..... 1.41.  
Carbon dioxide, percent..... 3.09.

**EXAMPLE 7**

55 This example illustrates the use of a crude grade of nonylphenols. It is seen that lower metal content results from the use of this phenol in place of the "commercial" grade of monononylphenol.

*Reagents Charged*

- 60 236 grams (1.0 mole, based on hydroxyl number) of technical nonylphenol  
472 grams of conventional paraffin oil (100 sec. at 100° F.)  
65 90 grams (1.0 mole) of formaldehyde (36% solution)  
25.2 grams (0.5 mole) of formic acid (88-90%)  
347 grams (1.1 moles) of barium hydroxide octahydrate

*Procedure*

70 The identical procedure was used as in the preparation of Example 1, except that a maximum dehydration temperature of 150° C. was used. Carbonation was done 75 conventionally at 200° C. for 2.5 hours.

## Product Analysis

|                            |                           |
|----------------------------|---------------------------|
| Barium, percent            | 13.31 (70% excess).       |
| Potentiometric base number | 112 (total), 23 (strong). |
| K.V. at 210° F., cs        | 17.44.                    |
| Formic acid, percent       | 2.64.                     |
| Carbon dioxide             | 3.01.                     |

## EXAMPLE 8

## Reagents Charged

|                                                              |
|--------------------------------------------------------------|
| 172 grams (0.5 mole) of dinonylphenol                        |
| 344 grams of conventional paraffin oil (100 sec. at 100° F.) |
| 25.5 grams (0.3 mole) of formaldehyde (36% solution)         |
| 174 grams (0.55 mole) of barium hydroxide octahydrate        |
| 28.3 grams (0.5 mole) of formic acid (88-90%)                |

The same procedure was used as described in Example 1 except that the maximum dehydration temperature was 150° C. Carbonation was conventional and was for 3.5 hours at 200° C.

## Product Analysis

|                            |                           |
|----------------------------|---------------------------|
| Barium, percent            | 2.47 (30% of theory).     |
| Potentiometric base number | 18 (total), 6.4 (strong). |
| K.V. at 210° C., cs        | 6.40.                     |

Another preparation using 1.0 mole of formaldehyde and 0.5 mole of formic acid per mole of dinonylphenol gave a barium content of 3.2% (37% of theory).

## EXAMPLE 9

## Reagents Charged

|                                                              |
|--------------------------------------------------------------|
| 110 grams (0.5 mole) of nonylphenol                          |
| 330 grams of conventional paraffin oil (100 sec. at 100° F.) |
| 174 grams (0.55 mole) of barium hydroxide octahydrate        |
| 28 grams (0.25 mole) of hydroxyacetic acid, 70% solution     |
| 42 grams (0.5 mole) of formaldehyde, 36% solution            |
| Carbon dioxide                                               |

## Procedure

The same procedure was used as described in Example 1, except that a maximum temperature of 150° C. was used during dehydration. The conventional method of carbonation was used by treating with carbon dioxide for 3 hours at 200° C.

## Product Analysis

|                            |                          |
|----------------------------|--------------------------|
| Barium, percent            | 11.2 (79% excess).       |
| Potentiometric base number | 80 (total), 24 (strong). |
| K.V. at 210° F., cs        | 12.90.                   |
| Glycolic acid, percent     | 1.75.                    |

Carbon dioxide, percent

## EXAMPLE 10

## Reagents Charged

|                                                              |
|--------------------------------------------------------------|
| 131 grams (0.5 mole) of dodecylphenol                        |
| 393 grams of conventional paraffin oil (100 sec. at 100° F.) |
| 174 grams (0.55 mole) of barium hydroxide octahydrate        |
| 12.6 grams (0.25 mole) of formic acid, 88-90%                |

42 grams (0.5 mole) of formaldehyde, 39% solution

## Procedure

The same as that used in Example 1, except that a maximum dehydration temperature of 150° C. was used.

## Product Analysis

|                                    |                          |
|------------------------------------|--------------------------|
| Barium, percent                    | 8.98 (58% excess).       |
| Potentiometric base number         | 65 (total), 48 (strong). |
| Kinematic viscosity at 210° F., cs | 24.13.                   |

## EXAMPLE 11

A portion of unfiltered material, prepared in Example 10, was carbonated by the conventional procedure for 5 hours at 200° C.

## Product Analysis

|                            |                          |
|----------------------------|--------------------------|
| Barium, percent            | 9.63 (70% excess).       |
| Potentiometric base number | 64 (total), 18 (strong). |

10 Kinematic viscosity at 210° F., cs

## EXAMPLE 12

In this example paraformaldehyde was substituted for the formaldehyde solution used in the preferred procedure.

## Reagents Charged

|                                                                                 |
|---------------------------------------------------------------------------------|
| 110 grams (0.5 mole based upon the theoretical molecular weight) of nonylphenol |
| 15 grams (0.5 mole) of paraformaldehyde                                         |
| 12.1 grams (0.25 mole) of formic acid, 88-90%                                   |
| 174 grams (0.55 mole) of barium hydroxide octahydrate                           |
| 330 grams of conventional paraffin oil (100 sec. at 100° F.)                    |
| Carbon dioxide                                                                  |

## Procedure

The same preparative method was used as described in Example 1, with the exception of the use of a maximum dehydration temperature of 150° C. This material was then carbonated by the usual method for 3 hours at 200° C.

## Product Analysis

|                            |                          |
|----------------------------|--------------------------|
| Barium, percent            | 12.2 (96% excess).       |
| Potentiometric base number | 75 (total), 22 (strong). |

35 Kinematic viscosity at 210° F., cs

## EXAMPLE 13(a)

This example illustrates successful utilization of a pre-formed alkylphenol-formaldehyde resin to give a complex salt product of the desired type. Ammonium hydroxide was used as the catalyst for the phenol-formaldehyde condensation reaction.

## Reagents Charged

|                                                                                   |
|-----------------------------------------------------------------------------------|
| 45 880 grams (4 moles based upon the theoretical molecular weight) of nonylphenol |
| 2460 grams of conventional paraffin oil                                           |
| 360 grams (4.0 moles) of formaldehyde, 36% solution                               |
| 20 ml. of ammonium hydroxide, 29.0% NH <sub>3</sub>                               |

## Procedure

All of the reagents were mixed in a five-liter, four-neck, round-bottom flask equipped with a mechanical stirrer, thermometer, nitrogen inlet tube and Dean-Stark water take-off with reflux condenser. The temperature was maintained in the range of 50-70° C. for one hour. Water was removed by distillation to a maximum temperature of 150° C. This temperature was held for two hours. The product was slightly viscous and yellow in color.

## Product Analysis

|                                    |        |
|------------------------------------|--------|
| Nitrogen, percent                  | 0.14.  |
| Specific gravity at 28° C.         | 0.900. |
| Kinematic viscosity at 210° F., cs | 4.78.  |

65 Hydroxyl No

74 (calculated=60).

Viscosity measurements on an oil blend of nonylphenol to give a comparable concentration gave the following results: Kinematic viscosity at 210° F., cs=3.87.

## EXAMPLE 13(b)

## Reactants Charged

|                                                                        |
|------------------------------------------------------------------------|
| 447 grams (0.5 mole) of condensation product prepared in Example 13(a) |
|------------------------------------------------------------------------|

174 grams (0.55 mole) of barium hydroxide octahydrate  
12.1 grams (0.25 mole) of formic acid, 88-90%  
Carbon dioxide

*Procedure*

The materials listed were charged into a two-liter, four-neck flask equipped with a mechanical stirrer, nitrogen inlet tube, thermometer, Dean-Stark water take-off tube and reflux condenser. The reaction mixture was stirred for one hour at a temperature of 80° C. to 100° C. for 30 minutes. Water was removed by distillation to a temperature of 150° C. This temperature was held for one hour to insure dryness. The reaction mixture was then treated by the conventional procedure with carbon dioxide for 3 hours at 200° C.

*Product Analysis*

Barium, percent..... 11.6 (86% excess).  
Potentiometric base number..... 81 (total), 27  
(strong).  
Kinematic viscosity at 210° F.,  
cs..... 8.24.  
Formic acid, percent..... 2.29.  
Carbon dioxide, percent..... 2.20.  
Specific gravity, at 28° C..... 1.041.

**EXAMPLE 14**

This example also illustrates the utilization of the preformed phenol-formaldehyde condensation product, but here formic acid is employed as the catalyst for the condensation. The formic acid remains in the reaction mixture and is ultimately incorporated into the complex salt product.

*Reagents Charged*

(A) 110 grams (0.5 mole based upon the theoretical molecular weight) of nonylphenol  
330 grams of conventional paraffin oil (100 sec. at 100° F.)  
12 grams (0.5 mole) of paraformaldehyde  
25.2 grams (0.5 mole) of formic acid (90%)  
(B) 174 grams (0.55 mole) of barium hydroxide octahydrate  
(C) Carbon dioxide

*Procedure*

All of the materials in group (A) were added to a one-liter, four-neck flask equipped with a mechanical stirrer, thermometer, nitrogen inlet tube, Dean-Stark take-off and reflux condenser. The reaction mixture was heated at 70-80° C. for one hour, to effect the phenol-formaldehyde condensation, then the hydroxide (B) was added. This mixture was dehydrated to a temperature of 150° C. and held at this temperature for one hour. The reaction mixture was then treated with carbon dioxide in the usual manner for 2 hours at 200° C.

*Product Analysis*

Barium, percent..... 10.6 (68% excess).  
Potentiometric base number..... 69 (total), 13 (strong).  
Kinematic viscosity at 210° F.,  
cs..... 9.19.

A product prepared in the same manner as Example 14, except that formaldehyde solution was substituted for the paraformaldehyde, gave the following analysis:

Barium, percent..... 10.5 (66% excess).  
Potentiometric base number..... 71 (total), 21  
(strong).

Kinematic viscosity at 210° F., cs..... 8.81.

**EXAMPLE 15**

This example illustrates the preparation of a complex salt of the invention by the reaction of formic acid with the carbonated product salt formed from the reaction of nonylphenol, formaldehyde and barium hydroxide.

*Reagents Charged*

220 grams (1.0 mole) of nonylphenol  
84 grams (1.0 mole) of formaldehyde (36% solution)  
347 grams (1.1 moles) of barium hydroxide octahydrate  
5 660 grams of conventional paraffin oil (100 sec. at 100° F.)

*Procedure*

The same procedure was used as in Example 1 except that the unfiltered product mixture was reacted with CO<sub>2</sub> by the conventional procedure at 200° C. for 5 hours and filtered.

To a 100-gram portion of the product thus obtained, 2.5 grams (0.5 mole) of formic acid (88-90%) was added dropwise over a twenty minute period at 120-150° C. to the filtered reaction product contained in a one-liter, four-neck, round-bottom flask equipped with a mechanical stirrer, dropping funnel, Dean-Stark water take-off, reflux condenser, thermometer and nitrogen inlet tube. 15 This reaction mixture was then heated to 200° C. to insure dryness. The product was cooled and filtered through a Buchner funnel (electrically-heated) to yield a viscous, yellowish-brown oil.

*Product analysis*

25 Barium, percent..... 13.1 (102% excess).  
Formic acid, percent..... 2.55.  
Carbon dioxide, percent..... 2.33.  
Potentiometric base number..... 94 (total), 26  
(strong).  
30 Kinematic viscosity at 210° F., cs..... 17.38.

**EXAMPLE 16**

*Reagents Charged*

35 110 grams (0.5 mole) of nonylphenol  
71.8 grams (1.1 moles) of potassium hydroxide, 86%  
45 grams (0.53 mole) of formaldehyde, 36% solution  
12.5 grams (0.25 mole) of formic acid, 88-90%  
330 grams of conventional paraffin oil (100 sec. at 40 100° F.)

*Procedure*

The same procedure was used as was shown in Example 1, except that a dehydration temperature of 150° C. was used.

*Product Analysis*

Potassium, percent..... 7.19 (100% excess).  
Potentiometric base number..... 101 (total), 69  
(strong).  
50 Kinematic viscosity at 210° F., cs..... 17.72.  
Formic acid, percent..... 4.01.

**EXAMPLE 17**

*Reagents Charged*

55 220 grams (1.0 mole) of nonylphenol  
91 grams (2.2 moles) of sodium hydroxide, 97.4%  
90 grams (1.05 moles) of formaldehyde, 36% solution  
25 grams (0.5 mole) of formic acid, 88-90%  
60 660 grams of conventional paraffin oil (100 sec. at 100° F.)

*Procedure*

This was the same as that used in Example 1, except 65 that the maximum dehydration temperature of 150° C. was used.

*Product Analysis*

Sodium, percent..... 3.70 (74% excess).  
Potentiometric base number..... 89.  
70 Kinematic viscosity at 210° F., cs..... 13.59.

The utility of the complex salts of this invention as lubricating oil additives has been demonstrated by comparative tests conducted on base lubricating oils alone and 75 these same oils blended with minor amounts of repre-

sentative product salts described in the preceding examples. The tests used were the Lauson Engine Test and the Catalytic Oxidation Test.

#### LAUSON ENGINE TEST

This test involves the operation of the single cylinder, 4-cycle, liquid-cooled Lauson engine under the following conditions: oil temperature, 270° F.; jacket temperature, 212° F.; speed, 1825 r.p.m.

The duration of the test is 100 hours and oil is added every 20 hours.

This test determines oil deterioration as primarily indicated by engine cleanliness. The engine which is clean at the start of the test is inspected after the test run for cleanliness of the rings, lands, ring grooves and piston skirt. Cleanliness ratings are made, based on a scale of from 100 to zero, a rating of 100 signifying a perfectly clean engine and a rating of zero representing the worst possible deposit condition.

The cleanliness rating obtained for the oil blend is compared to that found in a test employing the base oil alone, i.e., without addition of the additive.

In a test of a typical complex salt product of the invention, viz., the complex carbonated barium formate-nonylphenol-formaldehyde salt of Example 4, the base oil shows a cleanliness rating of 63, while the oil blend containing 2.45% (0.3 barium) of the complex salt showed a cleanliness rating of 85.

It has been found that besides their ability as detergents, the complex salts of the invention are also highly effective antioxidants for lubricating oils. This has been shown by subjecting several of the salt products to the Catalytic Oxidation Test.

#### CATALYTIC OXIDATION TEST (C.O.T.)

This test determines the effectiveness of an additive in preventing catalytic oxidation of an oil. The test procedure is as follows. In a 200 x 25 mm. test tube is placed a 25 cc. sample of test oil having immersed therein (a) 15.6 sq. in. of sandblasted iron wire, (b) 0.78 sq. in. of polished copper wire, (c) 0.87 sq. in. of polished aluminum wire and (d) 0.167 sq. in. of polished lead surface. The oil is heated to a temperature of 260° F. and maintained at this temperature, while drying air is being passed therethrough, at a rate of 18 liters per hour, for 40 hours. The results of the test are reported in terms of Stability Number of the additive. The Stability Number is the percentage of additive (in the oil) multiplied by 100, that reduces the N.N. (Neutralization Number) of the reference oil to a value of 2. Thus, the lower the additive Stability Number, the more effective the additive and vice versa. A Stability Number of 100 or less signifies a very good antioxidant.

The results of the C.O.T. tests are presented in Table I. The base oil used in all of the tests was an SAE 10 grade, solvent-refined, Pennsylvania oil (K.V. at 100° F.=35.75, K.V. at 210° F.=5.73).

TABLE I

| Additive (Ex. No.) | Percent metal in additive | C.O.T. test (Stability No.) |
|--------------------|---------------------------|-----------------------------|
| 1.                 | 11.69 (Ba)                | 85                          |
| 2.                 | 12.17 (Ba)                | 83                          |
| 4.                 | 12.27 (Ba)                | 80                          |
| 16.                | 7.19 (K)                  | 50                          |

It will be appreciated that the complex salt products, as provided by the process of this invention, are ordinarily concentrated oil solutions of the complex salts, these solutions containing from about 30% to about 70%, by weight, of the complex salts, the particular concentration depending upon the process conditions employed, includ-

ing the amount of solvent oil used in the process, etc. The amount of the product which is added to a petroleum fraction to provide a particular concentration of complex salt therein will, therefore, vary somewhat with a particular product. As a practical matter, however, differences in the products can be readily eliminated by standardization of process conditions and/or final adjustment of the product oil solutions to some standard salt content, as will be readily appreciated by those skilled in the art. Allowing for the usual variations in the salt contents of the product oil solutions, i.e., from about 30% up to about 70% of complex salt content, the amounts of the products to be utilized as additives in lubricating oil will range broadly from about 0.5% to about 30%, by weight, the usual amount being from about 2% to about 8%.

The additives of the invention may be used in lubricating oil compositions containing other additives designed to improve various characteristics of the oil, such as pour point depressants, viscosity index improvers, extreme pressure agents, other detergents, etc.

Although the present invention has been described herein by means of certain specific embodiments and illustrative examples, it is not intended that the scope thereof be limited in any way thereby, but only as indicated in the following claims.

This application is a division of application Serial No. 730,528, filed April 24, 1958, and now Patent No. 3,014,868.

#### What is claimed is:

1. A method for preparing a complex metal salt of an alkylphenol-formaldehyde condensation product which comprises (1) reacting about 1 mole of a monoalkyl-substituted phenol having from about 8 to about 18 carbon atoms in the alkyl substituent group thereof, in the presence of a hydrocarbon solvent, with (a) from about 0.5 to about 1.3 moles of formaldehyde, (b) from about 0.5 to about 1.0 mole of a carboxylic acid selected from the group consisting of formic acid and glycolic acid and (c) from about 0.85 to about 4.0 moles of a hydroxide of a metal selected from the group consisting of sodium, potassium, barium and strontium, the amount of said metal hydroxide being from about 1.70 to about 4.0 moles in the case of potassium and sodium hydroxides and from about 0.85 to about 2.0 moles in the case of barium and strontium hydroxides, at a temperature of about 40° C. to about 85° C., (2) heating the reaction mixture from step 1 at a temperature of at least about 150° C. to substantially completely dehydrate said mixture and (3) filtering off insoluble material.

2. A method for preparing a complex barium salt of an alkylphenol-formaldehyde condensation product which comprises (1) reacting an oil solution of a monoalkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of barium hydroxide, at a temperature of from about 40° C. to about 85° C., (2) heating the reaction mixture from step 1 at a temperature of at least about 150° C. to substantially completely remove water therefrom and (3) filtering off insoluble material.

3. A method for preparing a complex barium salt of an alkylphenol-formaldehyde condensation product which comprises (1) reacting an oil solution of a monoalkyl substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of barium hydroxide, at a temperature of from about 40° C. to about 85° C., (2) heating the reaction mixture from step 1 at a temperature of at least about 150° C. to substantially completely remove water therefrom, (3) treating the heated

reaction mixture from step 2 with carbon dioxide and (4) filtering off insoluble material.

4. A method for preparing a complex strontium salt of an alkylphenol-formaldehyde condensation product which comprises (1) reacting an oil solution of a mono-alkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of strontium hydroxide, at a temperature of from about 40° C. to about 85° C., (2) heating the reaction mixture from step 1 at a temperature of at least about 150° C. to substantially completely remove water therefrom and (3) filtering off insoluble material.

5. A method for preparing a complex strontium salt of an alkylphenol-formaldehyde condensation product which comprises (1) reacting an oil solution of a mono-alkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of strontium hydroxide, at a temperature of from about 40° C. to about 85° C., (2) heating the reaction mixture from step 1 at a temperature of at least about 150° C. to substantially completely remove water therefrom, (3) treating the heated reaction mixture from step 2 with carbon dioxide and (4) filtering off insoluble material.

6. A method for preparing a complex potassium salt of an alkylphenol-formaldehyde condensation product which comprises (1) reacting an oil solution of a mono-alkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 1.7 to about 4.0 moles of potassium hydroxide, at a temperature of from about 40° C. to about 85° C., (2) heating the reaction mixture from step 1 at a temperature of at least about 150° C. to substantially completely remove water therefrom and (3) filtering off insoluble material.

7. A method for preparing a complex sodium salt of an alkylphenol-formaldehyde condensation product which comprises (1) reacting an oil solution of a monoalkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 1.7 to about 4.0 moles of sodium hydroxide, at a temperature of from about 40° C. to about 85° C., (2) heating the reaction mixture from step 1 at a temperature of at least about 150° C. to substantially completely remove water therefrom and (3) filtering off insoluble material.

8. A complex metal salt of an alkylphenol-formaldehyde condensation product prepared by the method which comprises (1) reacting about 1 mole of a monoalkyl-substituted phenol having from about 8 to about 18 carbon atoms in the alkyl substituent group thereof, in the presence of a hydrocarbon solvent, with (a) from about 0.5 to about 1.3 moles of formaldehyde, (b) from about 0.5 to about 1.0 mole of a carboxylic acid selected from the group consisting of formic acid and glycolic acid and (c) from about 0.85 to about 4.0 moles of a hydroxide of a metal selected from the group consisting of sodium, potassium, barium and strontium, the amount of said metal hydroxide being from about 1.70 to about 4.0 moles in the case of potassium and sodium hydroxides and from about 0.85 to about 2.0 moles in the case of barium and strontium hydroxides, at a temperature of about 40° C. to about 85° C., (2) heating the reaction mixture from step 1 at a temperature of at least about 150° C. to substantially completely dehydrate said mixture and (3) filtering off insoluble material.

9. A complex barium salt of an alkylphenol-formaldehyde condensation product prepared by the method which comprises (1) reacting an oil solution of a monoalkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of barium hydroxide, at a temperature of from about 40° C. to about 85° C., (2) heating the reaction mixture from step 1 at a temperature of at least about 150° C. to substantially completely remove water therefrom and (3) filtering off insoluble material.

10. A complex barium salt of an alkylphenol formaldehyde condensation product prepared by the method which comprises (1) reacting an oil solution of a monoalkyl substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of barium hydroxide, at a temperature of from about 40° C. to about 85° C., (2) heating the reaction mixture from step 1 at a temperature of at least about 150° C. to substantially completely remove water therefrom, (3) treating the heated reaction mixture from step 2 with carbon dioxide and (4) filtering off insoluble material.

11. A complex strontium salt of an alkylphenol-formaldehyde condensation product prepared by the method which comprises (1) reacting an oil solution of a mono-alkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of strontium hydroxide, at a temperature of from about 40° C. to about 85° C., (2) heating the reaction mixture from step 1 at a temperature of at least about 150° C. to substantially completely remove water therefrom and (3) filtering off insoluble material.

12. A complex strontium salt of an alkylphenol-formaldehyde condensation product prepared by the method which comprises (1) reacting an oil solution of a mono-alkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 0.85 to about 2.0 moles of strontium hydroxide, at a temperature of from about 40° C. to about 85° C., (2) heating the reaction mixture from step 1 at a temperature of at least about 150° C. to substantially completely remove water therefrom, (3) treating the heated reaction mixture from step 2 with carbon dioxide and (4) filtering off insoluble material.

13. A complex potassium salt of an alkylphenol-formaldehyde condensation product prepared by the method which comprises (1) reacting an oil solution of a mono-alkyl-substituted phenol having from about 8 to about 18 carbon atoms in the alkyl substituent group thereof with (a) from about 0.5 to about 1.3 moles of formaldehyde, (b) from about 0.5 to about 1.0 mole of formic acid and (c) from about 1.7 to about 4.0 moles of potassium hydroxide, at a temperature of from about 40° C. to about 85° C., (2) heating the reaction mixture from step 1 at a temperature of at least about 150° C. to substantially completely remove water therefrom and (3) filtering off insoluble material.

14. A complex sodium salt of an alkylphenol-formaldehyde condensation product prepared by the method which comprises (1) reacting an oil solution of a mono-alkyl-substituted phenol having from about 8 to about 18 carbon atoms in the alkyl substituent group thereof with (a) from about 0.5 to about 1.3 moles of formalde-

hyde, (b) from about 0.5 to about 1.0 mole of formic acid and (c) from about 1.7 to about 4.0 moles of sodium hydroxide, at a temperature of from about 40° C. to about 85° C., (2) heating the reaction mixture from step 1 at a temperature of at least about 150° C. to substantially completely remove water therefrom and (3) filtering off insoluble material.

## References Cited in the file of this patent

## UNITED STATES PATENTS

2,736,701 Neff ----- Feb. 28, 1956

## FOREIGN PATENTS

440,110 Great Britain ----- Dec. 20, 1935